

# United States Patent Office

2,697,051

Patented Dec. 14, 1954

1

2,697,051

## TREATMENT OF TITANIUM METAL SURFACES

Svante Mellingen, Laurence Harbor, and Oliver W. Moles,  
Plainfield, N. J., assignors to National Lead Company,  
New York, N. Y., a corporation of New Jersey

No Drawing. Application September 17, 1952,  
Serial No. 310,132

7 Claims. (Cl. 134—30)

This invention relates to a method for pickling refractory metals. More specifically, it relates to a method for removing scale such as oxide coatings and the like from a titanium metal surface.

Titanium metal particularly at elevated temperatures has a strong affinity for oxygen, nitrogen, hydrogen and the like, and contact between the metal and these gases, both in the initial production steps and also in subsequent fabrication steps, often results in the formation of surface scale or coatings of the oxide, nitride, etc. When this type scale or coating is formed on such titanium metal products, the properties are often modified to such a degree that the products are no longer suitable for the purpose for which they had been intended. Furthermore, such surface scale adheres very tenaciously to the titanium metal and employment of pickling processes such as, for example, the acidic washes customarily used for the removal of scale from iron and steel have proved ineffective.

An object of this invention, therefore, is to provide a satisfactory process for removing such surface scale or coating from titanium metal in order to make the metal suitable for commercial utilization. Another object is to provide a quick and efficient method for reclaiming titanium from titanium metal products which are so contaminated. These and other objects will become obvious from the following more complete description of the instant invention.

Broadly speaking the instant invention contemplates a process for removing scale from a titanium metal surface which comprises treating said surface with a molten alkali metal polysulfide until said scale is loosened from said surface and removing said polysulfide and said loosened scale from said surface.

Alkali metal polysulfides which are suitable for employment in the instant process may be produced in a number of ways. For example, an alkali sulfide such as sodium sulfide ( $Na_2S$ ) may be combined with additional free sulfur to yield compositions corresponding to the general formula  $Na_2S_x$  where  $x$  is greater than unity. A particularly effective composition comprises either sodium or potassium polysulfides in which from about 0.1 to 5 parts of free sulfur are present in addition to that normally combined as  $Na_2S$  or  $K_2S$ . Mixtures of sodium and potassium polysulfides may also be used.

The polysulfide composition must be in the molten state. The temperatures at which such compositions melt vary considerably and is in part dependent upon the amount of free sulfur present. Satisfactory scale removal has been accomplished at temperatures of from about 250° C. to 500° C., naturally depending upon such factors as bath composition, apparatus size, design, etc.

When the titanium metal surface is treated with the molten polysulfide, the surface scale is loosened very rapidly, and generally, the metal product need be exposed to the action of the polysulfide for only a relatively short period of time. According to the instant process the treatment time should not exceed about ten minutes. Obviously shorter periods of contact may also be employed dependent upon the amount of scale and type of surface to be treated. However, it may be desirable on occasion to extend the treatment time beyond the ten minute period indicated above. For instance, the size of the article or the method of application of the polysulfide may be such that a longer time period would be more satisfactory. Accordingly, it has been found possible to buffer the action of the molten polysulfide by the addition of halide compounds such as, for example, the alkali and alkaline earth

2

metal halides including magnesium halides. These compounds in general are miscible with the polysulfides employed in the instant process. Obviously, the amount of halide compound which is used may vary and will depend on the degree of buffering action which is desired and upon the temperature to be employed. For practical utilization of such buffered polysulfide melts it has been found convenient to limit the amount of halide to that amount which will permit formation of a molten polysulfide-halide mixture at temperatures of from 250° C. to about 500° C. Furthermore, the addition of the buffer compound generally should be limited so as to permit the treatment time to be extended up to about one hour since longer periods are not particularly desirable in commercial operations.

In a further embodiment of the instant invention it may be desirable to rinse the metal surface from which the scale has been loosened with water to remove any remaining traces of loosened scale and polysulfide which may be present. The surface of the metal then possesses a fresh, clean metallic luster.

The actual method of treating the titanium metal surface with the molten polysulfide may, of course, vary; however, according to one preferred means, a molten bath of polysulfide is provided in which the titanium metal article which contains the surface scale may be appropriately immersed for a time sufficient to loosen said scale.

In order to describe the instant invention more clearly, the following examples are presented:

### Example I

A piece of 3/4" titanium bar stock, which had been hot rolled in an oxygen atmosphere and had been contaminated with an oxide scale, was immersed in a molten bath of sodium polysulfide, the composition of which corresponded generally to the formula  $Na_2S_3$  and which was heated at a temperature of about 350° C. The polysulfides immediately began to loosen the surface scale and after five minutes the bar of titanium metal was removed from the sulfide melt, rinsed with water and cooled to room temperature. The oxide coating had been completely removed and the metal bar had a fresh shiny metallic appearance.

### Example II

A titanium metal ingot which was covered with a surface scale of titanium oxide and titanium nitride was immersed in a molten bath comprising a mixture of sodium polysulfide and potassium polysulfide, the composition of which corresponded closely to the formula  $Na_2S_{1.3}K_2S$ . The ingot was permitted to remain in contact with the molten polysulfide mixture for a period of five minutes at a temperature of about 500° C. The ingot was then withdrawn from the polysulfide melt and subsequently cooled. Again, the surface scale had been completely removed, and the ingot possessed a bright and shiny metallic luster.

By the examples presented and by the preceding discussion, it has been demonstrated that according to the process of the instant invention, it is possible to effectively and swiftly remove surface scale such as oxide coatings from titanium metal by treating the metal surface with alkali metal polysulfide. This quick and efficient operation permits the reclamation of large quantities of titanium metal which would otherwise not be readily available for commercial utilization.

While this invention has been described and illustrated by the examples shown, it is not intended to be strictly limited thereto, and other variations and modifications may be employed within the scope of the following claims.

We claim:

1. A process for removing adherent scale from a titanium metal surface which comprises treating said surface with a molten alkali metal polysulfide until said scale is loosened from said surface and removing said polysulfide and said loosened scale from said surface.

2. A process for removing adherent scale from a titanium metal surface which comprises treating said surface with a molten alkali metal polysulfide for a period of not

more than about ten minutes to loosen said scale from said surface and thereafter removing said polysulfide and said loosened scale from said surface.

3. A process for removing adherent scale from the surface of a titanium metal product which comprises immersing said product in a molten alkali polysulfide for a period of not more than about ten minutes until said scale is loosened from said surface, substantially immediately thereafter withdrawing said product from said molten polysulfide, and rinsing with water to remove any remaining traces of loosened scale and polysulfide.

4. A process according to claim 1 wherein said polysulfide comprises sodium polysulfide.

5. A process according to claim 1 wherein said polysulfide comprises potassium polysulfide.

6. A process for removing adherent scale from a titanium metal surface which comprises treating said surface with a molten alkali metal polysulfide and a compound selected from the group consisting of alkali metal

halides and alkaline earth metal halides including magnesium halide until said scale is loosened from said surface and removing said polysulfide, said compound and said loosened scale from said surface.

5 7. A process for removing adherent scale from a titanium metal surface which comprises treating said surface with a molten alkali metal polysulfide and a compound selected from the group consisting of alkali metal halides and alkaline earth metal halides including magnesium halide for a period of not more than about one hour to loosen said scale from said surface and thereafter removing said polysulfide, said compound and said loosened scale from said surface.

15

**References Cited** in the file of this patent

The Canadian Mining and Metallurgical Bulletin for January 1951, Montreal, pages 25-28 (photostat in Div. 3) Ti Digest.